

## UNITED STATES PATENT OFFICE.

THORVALD OLSEN AALGAARD, OF GANDDALEN, NORWAY, ASSIGNOR TO CARL LARSEN, OF STAVANGER, NORWAY.

## MEANS FOR POLISHING METALS.

No Drawing.

Application filed August 11, 1921. Serial No. 491,568.

(GRANTED UNDER THE PROVISIONS OF THE ACT OF MARCH 3, 1921, 41 STAT. L., 1313.)

To all whom it may concern:

Be it known that I, THORVALD OLSEN AALGAARD, a subject of the King of Norway, residing at Ganddalén, Norway, have invented 5 a new and useful Means for Polishing Metals (for which I have filed application in Norway June 22, 1918, and in Denmark March 29, 1921), of which the following is a specification.

10 This invention relates to a metal polish containing cleaning and scouring substances and a luster-imparting substance consisting of onion juice.

15 As cleaning and scouring substances may be used soap, kerosene, water, carbonate of soda, and sand; but also other suitable ingredients may be used. The onion juice is of special importance as it renders a durable brilliancy to the metal.

20 I am aware that a composition containing onion juice has been used for washing clothes. This composition however has not contained scouring substances, and its purpose and the way of using it is entirely different from my invention.

The polish may be prepared in different ways and in any desired consistency, either as a liquid, a paste or a dry powder. It is preferably prepared in the following way: 30 50 gr. sliced onions are boiled for five minutes in 1000 gr. water, whereupon the onions are taken away, 1000 gr. of fine sand and 500 gr. of soap powder, comprising soap and sodium carbonate, are added, and the 35 mixture is then stirred until it has attained the consistency of a paste, whereupon it is boiled for five minutes. This paste is then dried and afterwards ground into a fine powder and is now ready for use.

It is applied in the following way: A cloth 40 is moistened with kerosene and is dipped into the powder, whereupon it is rubbed on the article to be polished. The article is then polished off with a dry cloth and dry powder. Instead of kerosene, water may be 45 used.

Another method of preparing the polish is the following:

500 gr. fine sand is mixed thoroughly with 50 gr. soap powder comprising soap and sodium carbonate, whereupon kerosene is added and the mixture is left quiet for half an hour. Then the surplus kerosene is poured off, and 35 gr. onion juice is added, whereupon the mixture is boiled for five 55 minutes, while being evenly stirred about. The stirring about is continued while the mixture is being cooled. When it is quite cold it has the consistency of a paste and is ready for use. 60

It is applied in a thin cover on a cloth and is rubbed on the article to be polished, whereupon the article is polished off with a dry, clean cloth. 65

I claim:

The herein described method of polishing metals which consists in applying to such metals a polish comprising cleaning and scouring substances and a luster imparting substance consisting of onion juice. 70

In testimony whereof I have signed my name in the presence of two subscribing witnesses.

THORVALD OLSEN AALGAARD.

Witnesses:

JONAS MELING,  
OLGA RISVOLD,